

1

3,201,241

DEVELOPER FOR DIAZO-TYPE PRINTING  
PLATES AND THE USE THEREOF

Johannes Munder and Hans Heiss, Wiesbaden-Biebrich, Gerhard Fritz, Wiesbaden, and Dieter Osswald and Hans Egon Heck, Wiesbaden-Biebrich, Germany, assignors, by mesne assignments, to Azoplate Corporation, Murray Hill, N.J., a corporation of New Jersey  
No Drawing. Filed July 11, 1961, Ser. No. 123,114  
Claims priority, application Germany, July 29, 1960,

K 41,325

26 Claims. (Cl. 96—49)

The present invention relates to a developer for photomechanical printing plates.

It is known to prepare planographic printing plates photomechanically by a process in which plates or foils made of metal or paper, e.g. aluminum, which have been provided with coatings of water-insoluble, light-sensitive substances, preferably consisting of diazo compounds, i.e. presensitized sheets, are illuminated on the light-sensitive side through a master and then the exposed coating is developed to an image by means of dilute aqueous alkaline solutions. Known developers for these coatings are, for example, aqueous solutions of di- or trisodium phosphate or of water-soluble organic bases of low concentrations. According to the type of the light-sensitive substance used, positive or negative printing images are obtained from the originals by the use of the alkaline developers, this being dependent upon whether it is the portions affected by the light or the portions not affected by the light that are removed by the developer.

As light-sensitive substances, quinone diazides have also been used, o-quinone diazides having found practical application for positive-working offset printing plates and p-quinone diazides for negative-working printing plates.

If coatings consisting of such compounds, or mixtures of such compounds, or mixtures of such compounds with resins are applied to a suitable support, e.g., an aluminum plate or paper foil, and are illuminated through a master, the coating is chemically changed in such a way that the portions affected by the light are less soluble in alkaline media of suitable concentration than are the portions unaffected by the light. Alkaline developer solutions of this kind, with which the portions unaffected by the light can be dissolved away, have consisted of aqueous solutions of alkali phosphates or silicates or of organic bases, such as ethanolamine. However, with these developer solutions the portions of the coating that have been illuminated are also partially dissolved away. For this reason, the length of the runs obtained with the printing plates produced is subject to variation according to the duration of the developer action.

A developer for photomechanical printing plates has now been found which consists of an aqueous solution which, in addition to an alkaline-acting substance, contains salts or oxides or hydroxides of the metals beryllium, mercury, calcium, strontium, barium, bismuth or lanthanum that are soluble in aqueous alkaline media and possibly also complex formers and/or water-soluble substances of higher molecular weight.

The alkaline-acting substances may be the basic substances used in the developer fluids for printing foils having diazo coatings, namely both organic and inorganic, weak and strong alkalis, the latter preferably in dilute form; examples are: water-glass, sodium metasilicate, potassium hydroxide, sodium hydroxide, diethylamine, triethylamine, ethanolamine, diethanolamine and triethanolamine. Mixtures of these alkalis may also be used.

Of the inorganic alkaline-acting substances, the silicates have proved particularly advantageous, particularly the

2

water-soluble alkaline metasilicates. Of the organic alkaline-acting substances, the lower aliphatic ones, particularly the hydroxy alkylamines, are preferred.

The salts, oxides or hydroxides of the metals, beryllium, mercury, calcium, strontium, barium, bismuth and lanthanum that are to be used in accordance with the invention are added in small quantities, namely about 0.001 percent to about 0.05 percent, preferably about 0.02 to 0.04 percent by weight. The effect depends chiefly on one or more of the cations of the metals mentioned above being present in the solution and the preference is for metals of the second group, particularly the alkaline earth metals. The cations are used, in addition to the oxides and hydroxides, in the form of their salts with inorganic and organic acids, provided they are readily, or at least moderately, soluble in alkaline aqueous solutions.

As the inorganic acids with which the salts are formed, the hydrohalides and nitric acid are preferred. As the organic acids, aliphatic mono and polycarboxylic acids such as formic acid, acetic acid, propionic acid, maleic acid, malonic acid, adipic acid and fumaric acid are primarily used.

To increase the solubility of the salts, oxides or hydroxides in alkaline media, complex formers may be added to the developer solution. In particular, complex formers which form 5 or 6-membered ring chelates such as hydroxyl compounds, hydroxy carboxylic acids, amino carboxylic acids, enolizable polycarbonyl compounds, nitrogen compounds containing hydroxyl and carboxyl groups, phenols, e.g., diethyl barbituric acid, citric acid, tartaric acid, saccharic acid, glycolic acid, adipic acid, ascorbic acid, Eriochrome Black R, Alizarin Yellow GG, salicylaldehyde, 2-hydroxyacetophenone, laevulinic acid, salicylic acid, Trilon B, acetylacetone, pyrocatechol, 5-benzene azo salicylic acid, 2-acetyl-1, 4-cresol, 6-acetyl-1, 3-cresol, dibenzoyl methane, and 8-hydroxy quinoline are suitable.

It is frequently advantageous for the complex formers to be added in a quantity in excess of that stoichiometrically required for the complex formation with the cation, as the coating treated therewith becomes more strongly anchored to the support. This results in an improved resistance of the developed image against the developer, which, in turn, causes higher runs of the printing plate. Water-soluble substances of high molecular weight which increase the viscosity can also be added to the developer solutions, e.g., polyglycols, such as polyethylene glycols having a molecular weight of 300 to 10000, carboxymethyl cellulose, cellulose ethers such as methyl cellulose, ethyl cellulose and polyvinyl alcohols. The developer solution should have a pH value between 10.5 and 12.2, preferably between 10.9 and 11.5.

The developer of the invention is suitable for the development of photomechanical printing plates consisting of a support coated with a light sensitive diazo coating. In particular, it is suitable for the development of printing plates of this type in which the light-sensitive coating, that has been exposed to light in known manner, consists at least in part of one or more p-quinone-diazide compounds of the general formula



in which  $R_1$  is an aromatic residue which may be substituted,  $R_2$  is a substituted or unsubstituted alkyl group or an aromatic, heterocyclic or aliphatic amino radical which is joined through the amino nitrogen atom to the group X and in which the residues may be substituted, 5  $R_3$  is hydrogen, alkyl, alkoxy or halogen, and X stands for  $\text{SO}_2$  or the CO-group.

Formulae of exemplary compounds are as follows:

FORMULA 1



FORMULA 2



FORMULA 3



FORMULA 4



4

FORMULA 5



FORMULA 6



FORMULA 7



FORMULA 8



FORMULA 9



Such p-quinone diazide compounds may be prepared, for example, in the following manner:

(1) 1-chloro-4-nitro-benzene-2-sulfochloride is reacted with an aromatic base to produce the 1-chloro-4-nitro-benzene-sulfaryl-amides. These intermediate products are condensed in solvents with aryl sulfonamides in the presence of copper powder and alkali carbonate, the chlorine in the 1-position then being replaced by the aryl sulfonamide residue. The nitro compounds thus obtained can be reduced by known processes, e.g. with sodium dithionite, and the amines thus obtained diazotized in water-miscible solvents, e.g. in a dimethylformamide/glacial acetic acid mixture. The iminoquinone diazides precipitate out for the most part in the form of sparingly soluble compounds or they can be precipitated by the addition of water.

(2) 4-nitro-1-amino-benzene-2-sulfonic acid is reacted with aromatic sulfo-chlorides and the 1-arylsulfamino-4-nitro-2-benzene sulfonic acids obtained are converted into the sulfochlorides which, in turn, are reacted with aromatic bases. The nitro compounds obtained are further processed as described above under 1.

The development of the exposed reproduction material with the alkaline developer liquid is in known manner, e.g., by immersion or, particularly, by wiping over with a cotton pad or a cloth soaked in the developer liquid. A brush may also be used for the application of the developer solution.

As a result of the addition of the metal cations in complex or non-complex form, the developer liquids described above, which contain about 0.3 to 5 percent by weight, preferably about 0.8 to 1.5 percent, of one or more of the alkaline substances listed, about 0.001 to 0.05 percent by weight, preferably 0.02 to 0.04 percent, of one or more of the salts, oxides or hydroxides of the metals mentioned, about 0.001 to 0.25 percent by weight, preferably about 0.07 to 0.1 percent, of complex formers and about C to 1.5 percent, by weight, preferably 0.2 to 0.8 percent, of additives such as polyglycols, enable a considerably greater number of prints to be prepared from printing plates developed with such a developer than from those developed using an otherwise identical developer solution to which the cations of the invention have not been added, because the image portions of the printing plate are to a much lesser extent attacked by the developer of the invention. For example, an exposed aluminum printing plate, the light-sensitive coating of which is applied in the form of a 1.3 percent solution of a compound corresponding to the following formula



by cast-coating upon an aluminum plate mounted on a rotating support and then dried, can be immersed in a solution containing 12 g. of sodium metasilicate  $\cdot 9\text{H}_2\text{O}$  per liter for only 5 minutes before the image disappears.

If 0.2 g. of barium hydroxide, or an equivalent quantity of a suitable barium complex salt, is added to the solution, the same plate can be treated for 60 minutes with the developer before the image undergoes an attack of equal intensity.

The invention will be further illustrated by reference to the following specific examples:

*Example 1*

5 An aluminum foil mounted on a rotating support was cast-coated with a thin, homogeneous, light-sensitive coating of a 1.3 percent solution in ethylene glycol monomethyl ether of the compound corresponding to Formula 2 above and then dried in a hot air current. The pre-sensitized material thus prepared was illuminated through a transparent master and then rubbed over with a cotton pad soaked in one of the solutions described below and then rinsed with water and dried. In this development process, the non-illuminated portions of the light-sensitive coating are removed.

10 The foil thus obtained, carrying a reversed image of the master, was inked up in the image portions with greasy ink and then prints were prepared in known manner.

20 As developer fluids for the treatment of exposed coatings, the solutions listed by way of example below have proved satisfactory.

(a) A solution of 10.0 parts by weight of sodium metasilicate  $\cdot 9\text{H}_2\text{O}$ , 0.3 part by weight of the calcium complex of Alizarin Yellow GG and 4.0 parts by weight of polyethylene glycol 6000 in 1000 parts by volume of water. The solution has a pH value of 11.2.

(b) A solution of 10.0 parts by weight of sodium metasilicate, 0.1 part by weight of calcium chloride and 3.0 parts by weight of polyethylene glycol 6000 in 1000 parts by volume of water. The solution has a pH value of 11.2.

(c) A solution of 20.0 parts by weight of sodium metasilicate  $\cdot 5\text{H}_2\text{O}$ , 0.3 part by weight of barium acetyl acetate and 3.0 parts by weight of polyethylene glycol 6000 in 1000 parts by volume of water. The solution has a pH value of 11.3.

*Example 2*

40 In the manner described in Example 1, an aluminum foil was coated with the light-sensitive compound corresponding to Formula 3 above and then developed to a printing plate. A printing plate having a reversed image of the master is obtained.

45 The developer solution used consisted of 10 parts by weight of sodium metasilicate  $\cdot 9\text{H}_2\text{O}$ , 0.3 part by weight of barium hydroxide and 0.3 part by weight of 2-acetyl-1,4-cresol in 1000 parts by volume of water.

*Example 3*

50 In the manner described in Example 1, an aluminum foil was coated with the light-sensitive compound corresponding to Formula 4 above and then developed to a printing plate. A printing plate having a reversed image of the master is obtained.

55 As a developer solution, either

(a) A solution of 10 parts by weight of sodium metasilicate  $\cdot 9\text{H}_2\text{O}$  and 0.3 part by weight of a mercury (II)-complex of 5-benzene-azosalicylic acid in 1000 parts by volume of water or

60 (b) A solution of 10 parts by weight of sodium metasilicate  $\cdot 9\text{H}_2\text{O}$  and 0.3 part by weight of calcium nitrate in 1000 parts by volume of water may be used.

*Example 4*

65 In the manner described in Example 1, an aluminum foil was coated with a solution of the compound corresponding to Formula 5 in ethylene glycol monomethyl ether in admixture with about equal parts of an alkali-soluble formaldehyde-cresol condensation product, a so-called novolak (Alnovol), and was then converted into a printing plate.

70 As a developer, a solution consisting of 10 parts by weight of sodium metasilicate  $\cdot 9\text{H}_2\text{O}$ , 0.3 part by weight of diethyl barbituric acid sodium salt and 0.3 part by

weight of strontium hydroxide in 1000 parts by volume of water was used.

*Example 5*

In the manner described in Example 1, an aluminum foil was coated with the light-sensitive compound corresponding to Formula 6 and then developed to a printing plate. A printing plate having a reversed image of the master is obtained.

As a developer, a solution of

(a) 4 parts by weight of sodium metasilicate  $\cdot 9H_2O$  and 0.3 part by weight of lanthanum oxide in 1000 parts by volume of water or

(b) 4 parts by weight of sodium metasilicate  $\cdot 9H_2O$ , and 0.3 part by weight of bismuth hydroxide and 0.3 part by volume of acetylacetone in 1000 parts by volume of water or

(c) 50 parts by volume of diethylamine and 300 parts by weight of calcium acetate in 1000 parts by volume of water may be used.

*Example 6*

In the manner described in Example 1, an aluminum foil is coated with the light-sensitive compound corresponding to Formula 7 and then developed to a printing plate.

A printing plate having a reversed image of the master is obtained.

As a developer, a solution of:

(a) 7 parts by weight of sodium metasilicate  $\cdot 9H_2O$  and 0.3 part by weight of beryllium oxide in 1000 parts by volume of water or

(b) 50 parts by volume of water glass, 0.3 part by weight of barium chloride and 0.3 part by volume of acetylacetone in 1000 parts by volume of water or

(c) 5 parts by weight of potassium hydroxide and 0.3 part by weight of strontium hydroxide in 1000 parts by volume of water may be used.

*Example 7*

1.3 parts by weight of the diazo compound corresponding to Formula 7 are dissolved in a mixture of 80 parts by weight of ethylene glycol monomethyl ether and 20 parts by weight of butyl acetate. A paper foil, which is provided on one side with a layer consisting of casein and clay hardened with formaldehyde, prepared in accordance with U.S. Patent 2,534,588, is coated with this solution on a rotating plate. The coating is well dried in a hot air current. The foil thus sensitized is illuminated through a transparent master with an arc lamp, as described in Example 1. The image produced is developed by wiping over with a cotton pad which has been soaked in a solution of the following composition: 7.5 parts by weight of sodium metasilicate  $\cdot 9H_2O$ , 0.3 part by weight of barium chloride, 0.3 part by volume of acetylacetone, and 1000 parts by volume of water. From a negative original a yellow-green positive image is obtained which is inked up with greasy ink and used a printing master. The resistance of the image to this developer is considerably greater than to a similar developer to which barium chloride and acetylacetone have not been added.

*Example 8*

In the manner described in Example 1, an aluminum foil was coated with the light sensitive compound corresponding to Formula 8 and then developed to a printing plate. A printing plate having a reversed image of the master is obtained.

The developer used consisted of a solution of 10 parts by weight of sodium metasilicate  $\cdot 9H_2O$  and 0.3 part by weight of strontium hydroxide in 1000 parts by volume of water.

*Example 9*

In the manner described in Example 1, an aluminum foil was coated with the light sensitive compound corresponding to Formula 9 and then developed to a printing plate. A printing plate having a reversed image of the master is obtained.

The developer used consisted of a solution of 10 parts by weight of sodium metasilicate  $\cdot 9H_2O$  and 0.3 part by weight of barium chloride in 1000 parts by volume of water.

It will be obvious to those skilled in the art that many modifications may be made within the scope of the present invention without departing from the spirit thereof, and the invention includes all such modifications.

What is claimed is:

1. A developer for planographic printing plates of the type including a light-sensitive diazo compound comprising an aqueous solution of at least of about 0.3 to 5 percent by weight one alkaline-acting substance selected from the group consisting of alkali metal compounds, alkylamines and hydroxy-alkylamines and about 0.001 to 0.05 percent by weight of at least one compound of an element selected from the group consisting of beryllium, mercury, calcium, strontium, barium, bismuth, and lanthanum, capable of cation formation in an aqueous medium.

2. A developer according to claim 1 including, in addition, a complex-forming compound.

3. A developer according to claim 1 including, in addition, a water-soluble compound of high molecular weight.

4. A developer according to claim 1 in which the alkaline-acting substance is a water-soluble alkali metal metasilicate.

5. A developer according to claim 1 in which the alkaline-acting substance is a hydroxy alkylamine.

6. A developer according to claim 1 in which the compound is selected from the group consisting of salts, oxides and hydroxides.

7. A developer according to claim 2 in which the complex-forming compound is one which forms a ring chelate.

8. A developer according to claim 3 in which the water-soluble compound of high molecular weight is a polyethylene glycol.

9. A process for developing a planographic printing plate of the type including a light-sensitive diazo compound which comprises treating the light-exposed coating thereof with a developer comprising an aqueous solution of about 0.3 to 5 percent by weight of at least one alkaline-acting substance selected from the group consisting of alkali metal compounds, alkylamines and hydroxy-alkylamines and about 0.001 to 0.05 percent by weight of at least one compound of an element selected from the group consisting of beryllium, mercury, calcium, strontium, barium, bismuth, and lanthanum, capable of cation formation in an aqueous medium.

10. A process according to claim 9 in which the developer includes, in addition, a complex-forming compound.

11. A process according to claim 9 in which the developer includes, in addition, a water-soluble compound of high molecular weight.

12. A process according to claim 9 in which the alkaline-acting substance is a water-soluble alkali metal metasilicate.

13. A process according to claim 9 in which the alkaline-acting substance is a hydroxy alkylamine.

14. A process according to claim 9 in which the compound is selected from the group consisting of salts, oxides and hydroxides.

15. A process according to claim 10 in which the complex-forming compound is one which forms a ring chelate.

16. A process according to claim 11 in which the water-soluble compound of high molecular weight is a polyethylene glycol.

17. A process according to claim 9 in which those por-

tions of the light-exposed coating which were not struck by light comprise a compound having the formula



in which R<sub>1</sub> is an aryl group, R<sub>2</sub> is selected from the group consisting of alkyl and aliphatic, aromatic and heterocyclic amino groups joined through the amino nitrogen atom to the group X, R<sub>3</sub> is selected from the group consisting of hydrogen, alkyl, alkoxy, and halogen, and X is selected from the group consisting of SO<sub>2</sub> and CO groups.

18. A process according to claim 9 in which those portions of the light-exposed coating which were not struck by light comprise a compound having the formula:



19. A process according to claim 9 in which those portions of the light-exposed coating which were not struck by light comprise a compound having the formula:



20. A process according to claim 9 in which those portions of the light-exposed coating which were not struck by light comprise a compound having the formula



21. A process according to claim 9 in which those portions of the light-exposed coating which were not struck by light comprise a compound having the formula



22. A process according to claim 9 in which those portions of the light-exposed coating which were not struck by light comprise a compound having the formula



23. A process according to claim 9 in which those portions of the light-exposed coating which were not struck by light comprise a compound having the formula



24. A process according to claim 9 in which those portions of the light-exposed coating which were not struck by light comprise a compound having the formula



11

25. A process according to claim 9 in which those portions of the light-exposed coating which were not struck by light comprise a compound having the formula:



5

10

26. A process according to claim 9 in which those portions of the light-exposed coating which were not struck by light comprise a compound having the formula:



25

30

35

12

## References Cited by the Examiner

## UNITED STATES PATENTS

|           |       |                |       |
|-----------|-------|----------------|-------|
| 2,062,273 | 11/36 | Reed et al.    | 96-49 |
| 2,564,414 | 8/51  | Whyzmuzis      | 96-49 |
| 2,732,299 | 1/56  | Morrison       | 96-49 |
| 2,759,817 | 8/56  | Schmidt et al. | 96-33 |
| 2,931,724 | 4/60  | Lantz          | 96-49 |
| 2,958,599 | 11/60 | Neugebauer     | 96-33 |
| 3,046,120 | 7/62  | Schmidt et al. | 96-33 |
| 3,046,121 | 7/62  | Schmidt        | 96-33 |

## FOREIGN PATENTS

922,506 1/55 Germany.

15 NORMAN G. TORCHIN, Primary Examiner.

PHILIP E. MANGAN, Examiner.

UNITED STATES PATENT OFFICE  
CERTIFICATE OF CORRECTION

Patent No. 3,201,241

August 17, 1965

Johannes Munder et al.

It is hereby certified that error appears in the above numbered patent requiring correction and that the said Letters Patent should read as corrected below.

Column 7, line 59, after "used" insert -- as --; line 73, for "if" read -- of --; column 8, line 19, strike out "of at least" and insert the same after "weight" in line 20, same column 8.

Signed and sealed this 15th day of February 1966.

(SEAL)

Attest:

ERNEST W. SWIDER

Attesting Officer

EDWARD J. BRENNER

Commissioner of Patents